

## UNITED STATES PATENT OFFICE

CAMILLE DREYFUS, OF NEW YORK, N. Y.

## PILE FABRIC

No Drawing.

Application filed May 22, 1930. Serial No. 454,834.

This invention relates to pile fabrics and particularly to pile fabrics containing yarns of organic derivatives of cellulose. An object of my invention is to produce pile fabrics having a pile of yarn containing organic derivatives of cellulose, which fabrics have a desirable lustre. Other objects of my invention will appear from the following detailed description.

10 Pile fabrics, such as velvets, containing a pile of ordinary yarns of organic derivatives of cellulose do not have the lustre and sheen often expected of such fabrics. I have found that this is due to the fact that yarns of organic derivatives of cellulose as ordinarily made are quite transparent, and that therefore when a fabric containing pile yarns of such material is viewed, the appearance is rather dull and lifeless due to the fact that 20 the light is not reflected sufficiently from the exposed ends of such pile, so that the back of the pile fabric is more conspicuous than it should be. I have found that if yarns of organic derivatives of cellulose of increased 25 opacity are employed as the pile, such pile yarns reflect the incident light sufficiently to impart a highly desirable lustre and sheen to the pile fabric.

In accordance with my invention, I 30 pare a pile fabric having a pile of yarns of organic derivatives of cellulose which yarns have an increased opacity, preferably caused by the presence of a finely divided pigment therein.

35 The pile of the fabric made in accordance with my invention contains yarns of any suitable organic derivative of cellulose such as organic esters of cellulose and cellulose ethers. Examples of such organic esters of cellulose are cellulose acetate, cellulose formate, cellulose propionate and cellulose butyrate, while examples of cellulose ethers are ethyl cellulose, methyl cellulose and benzyl cellulose. However I prefer to employ yarns of 40 cellulose acetate. The back of the fabric may be made of yarns of such organic derivatives of cellulose or it may be made of yarns of other fibres such as silk, reconstituted cellulose, cotton or wool. If desired, the back of 45 the fabric may be made of both yarns of or-

ganic derivatives of cellulose and yarns of such other fibres.

As stated in order to impart among other desirable properties the desired lustre, sheen, fullness and richness to the pile fabric, 55 the pile yarns of organic derivatives of cellulose should have an increased opacity. Preferably this increased opacity is caused by the presence therein of a finely divided pigment, preferably of white or light color, such as 60 zinc oxide, zinc sulphide, barium sulphate, calcium sulphate, strontium sulphate, barium phosphate, calcium phosphate, strontium phosphate, titanium dioxide, aluminum hydroxide, lead sulphate or nacreous materials 65 such as the silky or pearly form of mercurous chloride. These finely divided pigments may be incorporated in the yarn to be employed as the pile in any suitable manner. Thus the 70 finely divided pigment may be added to the spinning solution from which the yarns are formed. Another way of incorporating such finely divided material is to treat the yarn after its formation with an aqueous solution 75 of a soluble salt in the presence of a swelling agent for the particular organic derivative of cellulose and then to precipitate the pigment within the yarn by treatment with an aqueous solution of a salt or acid which forms an insoluble compound with the salt used in the 80 first treated solution. As an example of this, the yarn containing cellulose acetate may be treated with an aqueous solution of barium chloride in the presence of acetic acid, formic acid or lactic acid as a swelling agent, and 85 then treated with a solution of sulfuric acid or sodium sulphate to precipitate the barium sulphate therein. Alternatively, a soluble salt may be incorporated in the spinning solution from which the yarn is formed, and 90 the yarn or fabric then treated with a solution of a salt or acid that precipitates an insoluble compound in the yarn, either as a separate operation or in conjunction with a dyeing or 95 other finishing operation. However, I usually prefer to employ yarns formed from spinning solutions containing finely divided pigments in those cases where it is desired to have a greater surface lustre of the filaments or yarn. 100

Often in order to obtain a higher lustre in the pile fabric, it is desirable to cause the pile to occupy a position other than right angles to the plane of the back of the fabric.

5 Such pile may have an angle of from 0° to 75° to the plane of the fabric to produce a panne effect.

It is to be understood that the foregoing description is given merely by way of illustration and that many variations may be made therein without departing from the spirit of my invention.

Having described my invention, what I desire to secure by Letters Patent is:

16 1. A pile fabric having a pile comprising yarns of organic derivatives of cellulose having an opacity increasing material therein.

2. A pile fabric having a pile comprising yarns of cellulose acetate having an opacity increasing material therein.

3. A pile fabric having a pile comprising yarns of organic derivatives of cellulose having a finely divided pigment therein.

25 4. A pile fabric having a pile comprising yarns of cellulose acetate having a finely divided pigment therein.

5. A pile fabric having a pile comprising yarns of organic derivatives of cellulose having a finely divided pigment therein, which pile is not at right angles to the plane of the

30 surface of the fabric.

6. A pile fabric having a pile comprising yarns of cellulose acetate having a finely divided pigment therein, which pile is not at

35 right angles to the plane of the surface of the fabric.

In testimony whereof, I have hereunto subscribed my name.

CAMILLE DREYFUS.

40

45

50

55

60

65